

# United States Patent

Runevall et al.

[15] 3,693,394

[45] Sept. 26, 1972

[54] PROCESS IN CONTINUOUS  
EXTRUSION OF METALS AND THE  
LIKE

[72] Inventors: Agar Evald Runevall, Tranvagen 67,  
Segeltorp; Bror Hansson, Kar-  
lavagen 97, Stockholm, both of  
Sweden

[22] Filed: Nov. 12, 1970

[21] Appl. No.: 88,707

[30] Foreign Application Priority Data

Nov. 17, 1969 Sweden 15710/69

[52] U.S. Cl. 72/262

[51] Int. Cl. B21c 29/00

[58] Field of Search 72/262; 18/30 SM

[56]

## References Cited

### UNITED STATES PATENTS

|           |        |                       |          |
|-----------|--------|-----------------------|----------|
| 2,743,812 | 5/1956 | Ljungberg .....       | 72/262   |
| 2,593,265 | 4/1952 | Chase et al. ....     | 72/262   |
| 3,055,053 | 9/1962 | Livingston et al..... | 18/30 SM |
| 2,172,651 | 9/1939 | Dunsheath.....        | 72/262   |

Primary Examiner—Richard J. Herbst

Attorney—Sommers & Young

[57] ABSTRACT

Metal and the like is extruded by means of a screw press including a power zone and extrusion die means. On leaving the power zone, the metal is heated to facilitate its passage from the screw to and through the die means.

5 Claims, 9 Drawing Figures



FIG.1



FIG.2



FIG.3



FIG.4



Agar Evald Runewall  
 Bror Hansson  
 Inventors

by Sommers & Young  
 Attorneys

FIG.5



Agar Evald Runewall  
Bror Hansson  
Investors  
By Drimmers & Young  
Attorneys

PATENTED SEP 26 1972

3,693,394

SHEET 3 OF 3



FIG. 6A

FIG. 6C



FIG. 6B



FIG. 6D

Agar Evald Runewall  
Bror Hansson

Inventors

by Sommers & Young  
Attorneys

## PROCESS IN CONTINUOUS EXTRUSION OF METALS AND THE LIKE

### BACKGROUND OF THE INVENTION

The present invention relates to a process for the continuous extrusion of metals and the like by means of screw presses.

During the extrusion of metals, for instance lead, by means of a screw press considerable pressure is necessary to force the lead through the die block and the dies of the press. On account of the fact that a pressure at a couple of thousand atmospheres is required, the friction losses in the die block will be considerable. This applies to the sliding frictions between lead and the steel faces of the screw and the die block respectively, as well as to the internal friction losses within the lead itself, when this is reshaped in the press head and in the dies. The friction losses which are taken from the kinetic energy of the metal cause the pressure to be reduced towards the dies, whereby the efficiency of the machine is limited. Furthermore this has the effect that the usability of such a screw press will be strongly reduced with respect to hard lead alloys or other hard metals such as aluminum.

The processes thus far known for extrusion of metal and the like have not been entirely successful in eliminating the above disadvantages. Thus it is the object of the present invention to achieve an improved process for continuous extrusion, which has a better efficiency and a wider field of application than previously known processes.

### SUMMARY OF THE INVENTION

In the process of the invention metals and the like are extruded continuously by means of screw presses. In their power zones the rotational energy of the screw is transferred to the metal in the form of high pressure and an axial forward movement of the metal. The advantages of the invention are achieved by causing the metal, as soon as possible after it has left the power, to be heated whereby internal friction in the lead is reduced by the elevated temperature. This reduction in friction makes the passage of the metal from the screw tip to the shaping dies easier.

The metal can be heated by supplying electric heat, hot gas or liquid or combustion gases in the interior of the screw tip and/or in a wedge-shaped member dividing the lead and located immediately above the tip of the screw.

According to another embodiment of the invention, the heating can be achieved by means of inner friction in the metal mass itself. The threads of the top of the screw are, for this purpose, shaped so that they constantly knead the metal mass during the rotation of the screw.

### BRIEF DESCRIPTION OF THE DRAWINGS

The invention will be described more in detail below with reference to the accompanying drawings, in which:

FIG. 1 shows a known screw press for extruding lead tubes;

FIG. 2 is a side view of a lead dividing member located in the die block of the screw press in FIG. 1;

FIG. 3 is a section along the line 3—3 of FIG. 2;

FIG. 4 is a section along the line 4—4 of FIG. 2;

FIG. 5 is a graph showing the shearing strength as a function of the temperature of pure lead (A) and of a lead alloy (B);

FIG. 6A—6D inclusive show some possible designs of the screw tip of the press which operate to knead the metal mass according to an embodiment of the invention, FIGS. 6B and 6D being plan view of the screw structures shown in FIGS. 6A and 6C respectively.

### DESCRIPTION OF THE PREFERRED EMBODIMENTS

FIG. 1 shows a known screw press for extrusion of a lead tube with a screw 2 located in a screw housing 4, whose interior walls are provided with longitudinal grooves (not shown). Molten lead is supplied through an inlet 3, and while being cooled the lead is moved upwards due to the rotary motion of the screw 2. When the lead has been cooled below its melting point, it enters during its motion upwards the so-called power zone of the screw press, which is the zone where the lead is further cooled and in which the pressure in the solid lead mass is built up, and in which the rotational energy of the screw is thus transferred to the lead mass in the form of high pressure and upward motion of the lead. The lead mass is moved further upwards, is divided by a lead dividing member 9 located in a die block 5 and is extruded through dies 6 and 7 to form a pipe 8. The lead dividing member 9 is shown in detail in FIG. 2, 3 and 4. The rotational energy of the screw will thus be transferred to this solid nut and the nut is forced upwards.

The pressure necessary for the extrusion is thus built up in the power zone of the screw press, in which a strong nut of solid lead is formed around the screw in order that great energy might be transferred to the lead mass via the nut.

The energy which can be transferred to the nut from the screw depends on the temperature of the lead. In FIG. 5 the curve A shows the shearing strength of pure lead depending on the temperature, and the curve B relates to a lead alloy. Obviously the temperature of the lead in the power zone, where the nut is formed, should be as low as possible.

The amounts of energy which are converted in a normal Hansson-Robertson lead press, during extrusion of tubes, will be better appreciated by reference to the following table:

|                                                                                                                                                   | Pure lead | Alloyed lead |
|---------------------------------------------------------------------------------------------------------------------------------------------------|-----------|--------------|
| Production per minute                                                                                                                             | 40 kg     | 20 kg        |
| For melting this amount of lead in the melting pot and raising its temperature to 400° C an effect is required of.....                            | 40 kW     | 20 kW        |
| For cooling (in the power zone of the press) of the lead to solidification and about 150° C it is necessary to remove from the lead approx. ..... | 38 kW     | 19 kW        |
| For extrusion the screw has to (in the power zone) transfer to the lead an effect of (measured value) approx. ....                                | 40 kW     | 60 kW        |

The power transferred by the screw to the lead for extrusion is thus large enough to melt the lead, and in order to achieve a sufficiently low temperature in the power zone special cooling must take place there, for instance by means of cooling liquid circulating in channels 10 in the screw housing 4 (see FIG. 1) or in channels in the screw itself. Through this cooling good strength of the nut formed by the lead in the power zone is secured.

During the passage of the lead mass from the power zone through the die block to the from dies, large losses of energy in the form of friction arise. In the process of the invention these shearing are reduced by heating the lead after it has left the power zone. As appears from FIG. 5, the shearing strength is considerably reduced in this way and consequently also the inner friction. If the inner friction and the pressure needed for extrusion of the lead is thus reduced, the friction losses between the lead and the steel parts of the die block are also reduced.

The heat can be supplied to the lead for instance in the form of electric heat, hot gas or liquid, or combustion gases in the interior of the screw tip 2 and/or the lead dividing member 9. No example of this is shown on the drawings.

The heat may also be supplied to the lead in the form of friction heat. The upper threads of the screw tip above the power zone may be provided with irregularities which, during the rotation of the screw while the threads carry the lead upwards, knead the lead so that it is heated through internal and/or external friction. FIGS. 6A—B and 6C—D, respectively, show two examples of such thread configurations the uppermost thread of the screw tip being provided with cuttings and oblique grooves on the edge of the thread. These cuttings and grooves are shaped so that metal does not accumulate therein. Accumulation of metal should be avoided especially at extrusion of alloys, as a segregation of the alloying components may arise in a remaining metal quantity, which might later be carried along and cause quality errors in the extruded metal product. It is advantageous if the screw tip is so designed that the lead is here reshaped and kneaded in such a way that the heating is substantially achieved by internal friction in the whole lead mass and not through surface friction between lead and screw, which might easily cause concentration of alloying components where the alloy is rubbed against steel.

Another advantage of heating by means of kneading from the rotating screw, is that such heating is direct proportional to the speed of the screw and thus also proportional to the extruded quantity of lead, and the heating ceases automatically when the machine is stopped.

This way of improving the extruding ability of screw

presses can of course with advantage also be used for such screw presses which lack a die block, but instead have inner dies placed in a spider which centers the inner die in the outer die. The spokes of such a spider offer a resistance corresponding to the resistance of a die block, such as shown in FIG. 1.

Thanks to the heating the lead will flow easier through the complicated nooks in the die block towards the shaping dies. There it may, however, be suitable to cool the lead again according to known methods so that it, by cold working, is given good mechanical properties at the very moment of extrusion.

With reference to FIG. 5 it has been mentioned that the internal friction of lead and lead alloys is strongly dependent on the temperature of the lead. Investigations show, however, that the sliding friction metal/steel is not so strongly dependent on the temperature or on the kind of alloy being used. It is, however, emphasized that if the internal friction is reduced with the process of the invention, it will be possible to operate with a lower pressure, and then the friction between steel and metal will also be reduced, as this sliding friction metal to steel is proportional to the pressure.

What we claim is:

1. A process for the extrusion of metal and the like by means of a screw press having a power zone in which the rotational energy of the screw is transferred to the metal in the form of pressure and axial forward motion, comprising the step of heating the metal as soon as possible after it has left the power zone, whereby the friction between the metal and screw is reduced by the increased temperature of said metal to facilitate the passage of the metal from the screw to and through the dies which shape the extruded product, said metal heating step being effected by reshaping and kneading the metal at the tip of the screw downstream of said power zone to produce heat in the form of internal friction within the metal.
2. The process of claim 1 wherein the internal friction in the metal mass is achieved by shaping the threads of the screw at the screw tip so that, during the rotation of the screw, said shaped threads constantly reshape and knead the metal mass.
3. The process of claim 1 wherein said kneading is achieved by means of depressions and/or enlargements on the core or threads of the screw tip.
4. The process of claim 2 wherein the friction heat produced at the screw tip is carried away by means of a coolant flowing within the screw.
5. The process of claim 3 wherein the depressions and/or enlargements on the threads or core of the screw are even in configuration, streamlined, and so directed that the metal cannot accumulate and remain therein.

\* \* \* \* \*